

[54] **ALUMINUM CORROSION INHIBITOR**

[75] Inventor: **Billy R. Keeney**, Duncan, Okla.

[73] Assignee: **Halliburton Company**, Duncan, Okla.

[22] Filed: **June 16, 1971**

[21] Appl. No.: **153,841**

**Related U.S. Application Data**

[63] Continuation of Ser. No. 783,117, Dec. 11, 1968, abandoned.

[52] **U.S. Cl.** ..... **106/14, 252/146, 252/148, 252/151, 252/388, 252/390, 252/395**

[51] **Int. Cl.** ..... **C09d 5/08**

[58] **Field of Search** ..... **106/14; 252/79.1, 79.2, 252/79.4, 8.55, 389, 390, 396**

[56] **References Cited**

**UNITED STATES PATENTS**

3,404,094 10/1968 Keeney ..... 252/396 X

3,319,714 5/1967 Knox ..... 252/8.55 X  
3,382,179 5/1968 Keeney et al. ..... 252/396 X

*Primary Examiner*—Harry Wong, Jr.

*Attorney, Agent, or Firm*—Thomas R. Weaver; John H. Tregoning

[57]

**ABSTRACT**

An aluminum corrosion inhibitor for use with aqueous acids. The inhibitor may take the form of a mixture of an anionic surface active agent and one or more acetylenic compounds, which mixture may further contain one or more of the following materials: nitrogen base compounds, non-acetylenic alcohols and aldehydes.

**18 Claims, No Drawings**

## ALUMINUM CORROSION INHIBITOR

This is a Continuation of application Ser. No. 783,117, filed Dec. 11, 1968, now abandoned.

## BACKGROUND OF THE INVENTION

## 1. Field of the Invention

The present invention relates generally to corrosion inhibitors and methods for inhibiting the corrosion of metals, and more particularly, but not by way of limitation, to an aluminum corrosion inhibitor for use with aqueous acids, and to methods for inhibiting the corrosion of aluminum by aqueous acids.

## 2. Description of the Prior Art

Prior known compositions for the inhibition of corrosion of aluminum surfaces when contacted with aqueous acids have been employed with varying degrees of success. A failing of these prior art corrosion inhibiting compositions is that they cease to be effective after relatively short periods of time or breakdown under high temperature conditions, that is, temperatures in the range of from 125° to 175°F., or higher. A further failing of these prior art compositions is that they are not effective to a comparable degree for substantially all commonly used aluminum alloys.

## SUMMARY OF THE INVENTION

The present invention relates to new and useful compositions which may be employed in acid solutions to decrease or inhibit the corrosion of aluminum in contact with the acid solutions. The present invention provides a corrosion inhibitor for inhibiting the corrosion of aluminum and alloys thereof by aqueous acids, which inhibitor comprises an anionic surface active agent and an acetylenic compound. The invention further provides a method for inhibiting the corrosion of aluminum and alloys thereof.

The present invention is particularly useful in cleaning aluminum with aqueous acids such as in the removal of scale from aluminum heat exchangers, tanks, pipes, etc., with dilute hydrochloric acid and inhibiting corrosion of aluminum tanks, pipes, etc., which must contain dilute acids.

It is therefore an object of the present invention to provide an inhibitor composition and a method of inhibiting corrosion of aluminum surfaces when such surfaces are contacted by aqueous acids.

Another object of the present invention is the provision of an inhibitor composition and a method of inhibiting the corrosion of aluminum surfaces when contacted with aqueous acids, which composition and method are effective at low temperatures as well as high temperatures.

A further object of the present invention is to provide an inhibitor composition and a method of inhibiting the corrosion of aluminum and alloys thereof when contacted with acid solutions, especially hydrochloric acid at high temperatures for relatively long periods of time.

Yet a further object of the present invention is to provide an inhibitor composition and a method of inhibiting aluminum and alloys thereof when contacted with acid solutions whereby a comparable degree of corrosion inhibition may be obtained for most commonly used aluminum alloys.

These and other objects and advantages of the present invention will become readily apparent from the

description of the invention and examples which follow.

## DESCRIPTION OF THE PREFERRED EMBODIMENTS

It has been discovered that an anionic surface active agent and an acetylenic compound, in particular amounts of each, provides a composition having superior aluminum corrosion inhibiting properties when 10 added in proper order in small quantities to an acid solution constituting the corrodent. In addition, an anionic surface active agent together with a synergistic blend of an acetylenic compound and a non-acetylenic alcohol; or one or more acetylenic compounds, a nitrogen base compound and one or more non-acetylenic alcohols; or one or more acetylenic compounds, a nitrogen base compound and an aldehyde or a solution 15 of aldehyde in alcohol; when added to a corrodent acid solution in particular quantities and in particular order provide compositions having superior aluminum corrosion inhibiting properties. The relative amounts of the acetylenic compound, non-acetylenic alcohol, nitrogen base compound and aldehyde may vary over a wide 20 range. Furthermore, it has been found that one of the preferred compositions described above may be used in 25 preference to another to obtain the best corrosion inhibiting properties, depending on the particular aluminum alloy to be protected, the temperatures to be encountered, and the strength or concentration of the acid corrodent. In general, the anionic surface active agent concentration in the corrosion inhibitor may vary 30 from about 15% to 35%. However, lower and higher concentrations will still be effective.

In the preferred form of the invention the anionic surface active agent is a saturated hydrocarbon sulfonate having the general formula  $RSO_3X$  with R being a  $C_8$  to  $C_{25}$  saturated hydrocarbon chain and X being an alkali metal or ammonium. The sulfonate is made by treating a saturated hydrocarbon (aliphatic or cycloaliphatic) of some predetermined chain length with sulfur dioxide and chlorine in the presence of actinic light. Gamma radiation and certain catalysts can be substituted for the actinic light. This forms a hydrocarbon sulfonyl chloride which is subsequently neutralized 40 with an alkali metal hydroxide or ammonium hydroxide. The preferred material has the formula  $C_{13}H_{27}SO_3Na$  and is made by gassing a C-13 straight chain saturated hydrocarbon (aliphatic) to a specific 45 gravity of 0.91 to 0.97 before neutralization. The anionic surface active agent  $C_{13}H_{27}SO_3Na$  is sometimes referred to herein after as CRA. U.S. Pat. No. 2,999,812 illustrates a method of preparing this preferred surface active agent.

Some examples of other anionic surface active agents which may be employed in the present invention are alkyl taurate, alkyl phosphate, alkyl sulfate, alkyl sulfonate, and alkyl aryl sulfonate.

In the preferred form of the invention, acetylenic alcohols having an ethynyl hydrogen on the acetylenic group are employed as the acetylenic compound component. Some examples of acetylenic alcohols or compounds which may be employed in the present invention are: hexynol, dimethylhexynol, dimethylhexynediol, dimethyloctynediol, methylbutynol, methylpentynol, ethynyl cyclohexanol, 2-ethylhexanol, phenylbutynol, and tertiary acetylenic glycol. Other acetylenic compounds which can be employed in accor-

dance with the present invention are for example, butynediol, 1-ethynylcyclohexanol, 3-methyl-1-nonyn-3-ol, 2-methyl-3-butyn-2-ol, also 1-propyn-3-ol, 1-butyn-3-ol, 1-pentyn-3-ol, 1-heptyn-3-ol, 1-octyn-3-ol, 1-nonyn-3-ol, 1-decyn-3-ol, 1-(2, 4, 6-trimethyl-3-cyclohexenyl) -3-propyne-1-ol, and in general acetylenic compounds having the general formula



wherein R is an alkyl, phenyl, substituted phenyl or hydroxylalkyl radical or —H, and the alpha R's may be joined together to form a cyclohexyl ring.

Acetylenic sulfides having the general formula



can also be employed in the present invention in lieu of the acetylenic alcohols. Examples of these are di-paraparagyl sulfide, bis (1-methyl-2-propynyl) sulfide and bis (2-ethynyl-2-propyl) sulfide.

The non-acetylenic alcohols suitable for use in the present invention have the general formula ROH, wherein R is either an alkyl group or a ketone group. Some examples of these alcohols are diacetone alcohol, normal propanol, isopropanol, ethanol, methanol, ethylene glycol, diethylene glycol, propylene glycol, dipropylene glycol, hexylene glycol, and 1,5-pentanediol.

The nitrogen or ammonia base compounds that may be employed in accordance with the present invention are those amines such as mono-, di- and trialkyl amines having from two to six carbon atoms in each alkyl moiety, as well as the six-membered n-heterocyclic amines, for example alkyl pyridines and mixtures thereof. These compounds include such amines as ethylamine, diethylamine, triethylamine, propylamine, dipropylamine, tripropylamine, mono-, di-, and tributylamine, mono-, di-, and tripentylamine, mono-, di-, and trihexylamine, and isomers of these, such as isopropylamine, tertiary butylamine, etc. The suitable nitrogen compounds also include alkyl pyridines having from one to five nuclear alkyl substituents per pyridine moiety, with such alkyl substituents having from one to 12 carbon atoms. The pyridines are preferred which have an average of six carbon atoms per pyridine moiety, e.g., a mixture of high boiling tertiary-nitrogen-heterocyclic compounds such as HAP (high alkyl pyridines), Reilly 10-20 base and alkyl pyridines HB.

The aldehydes which may be used in accordance with the present invention include alkyl aldehydes, aryl aldehydes, alkylaryl aldehydes. The aldehydes may be substituted with non-deleterious substituents, such as hydroxyl group, and may be saturated or unsaturated. Suitable aldehydes include formaldehyde, benzaldehyde, butyraldehyde, B-hydroxybutyraldehyde (aldol) propionaldehyde and glyoxal. The aldehyde may be used alone or in a suitable solvent such as alcohol.

Anionic surface active agents of this invention are generally not compatible with the other compounds employed in the corrosion inhibiting composition. Therefore, the corrosion inhibitor composition should be made up in two parts, the first part composed of the anionic surface active agent, and the second part composed of the acetylenic compound, or a blend of the acetylenic compound and the other compounds disclosed above. The acid solution containing the corro-

sion inhibitor composition may then be prepared by preparing the desired acid solution, then combining the surface active agent with the acid solution and mixing it thoroughly, and then combining the acetylenic compound or blend of acetylenic compound and other compounds with the acid solution and mixing thoroughly. Another method for preparing an acid solution containing the corrosion inhibitor composition of the present invention is to combine the surface active agent with a proper amount of water stirring it thoroughly, then combining the acetylenic compound or blend of acetylenic compound and other compounds with the water and stirring it thoroughly, and thereafter combining a proper amount of acid to complete the desired acid solution.

On a basis of a volume of 100 per cent, a preferred composition of the present invention is comprised as follows:

|                              | Per Cent |
|------------------------------|----------|
| Anionic Surface Active Agent | 15-35    |
| Acetylenic Compound          | 65-85    |

Another preferred composition of the present invention is comprised as follows:

|                              | Per Cent |
|------------------------------|----------|
| Anionic Surface Active Agent | 15-35    |
| Acetylenic Compound          | 30-60    |
| Nitrogen Compound            | 0-8      |
| Non-acetylenic Alcohol       | 10-50    |

Yet another preferred composition of the present invention is comprised as follows:

|                              | Per Cent |
|------------------------------|----------|
| Anionic Surface Active Agent | 15-35    |
| Acetylenic Compound          | 30-60    |
| Nitrogen Compound            | 0-8      |
| Aldehyde                     | 10-30    |
| Non-acetylenic alcohol       | 5-15     |

The non-acetylenic alcohol not only acts as a diluent and/or solubilizer, but also contributes to the corrosion inhibiting effectiveness of the novel composition for some applications. The nitrogen compound also contributes to the corrosion inhibiting effectiveness of the novel composition for some aluminum alloys as does the aldehyde.

On a basis of a volume of 100 per cent, a more specific preferred composition, sometimes referred to herein as composition A, of the present invention is as follows:

| Compound      | Composition A<br>Parts by<br>Volume | Per Cent<br>By Volume |
|---------------|-------------------------------------|-----------------------|
| CRA           | 1.0                                 | 30.0                  |
| Ethyl Octynol | 2.33                                | 70.0                  |

Another preferred specific composition, sometimes referred to herein as composition B is as follows:

| Compound | Composition B<br>Parts by<br>Volume | Per Cent<br>By Volume |
|----------|-------------------------------------|-----------------------|
| CRA      | 1.0                                 | 30.0                  |

| Compound          | Composition B<br>Parts by<br>Volume | Per Cent<br>By Volume |
|-------------------|-------------------------------------|-----------------------|
| Ethyl Octynol     | 1.6                                 | 49.0                  |
| Diacetone Alcohol | 0.7                                 | 21.0                  |

Yet another preferred composition, sometimes referred to herein as composition C is as follows:

| Compound           | Composition C<br>Parts by<br>Volume | Per Cent<br>By Volume |
|--------------------|-------------------------------------|-----------------------|
| CRA                | 1.00                                | 25.0                  |
| Propargyl Alcohol  | 1.38                                | 34.4                  |
| Ethyl Octynol      | 0.14                                | 3.4                   |
| Alkyl Pyridines HB | 0.11                                | 2.8                   |
| Diacetone Alcohol  | 1.38                                | 34.4                  |

Still another preferred composition, sometimes referred to herein as Composition D is as follows:

| Compound                          | Composition D<br>Parts by<br>Volume | Per Cent<br>By Volume |
|-----------------------------------|-------------------------------------|-----------------------|
| CRA                               | 1.00                                | 25.00                 |
| Propargyl Alcohol                 | 1.36                                | 33.94                 |
| Ethyl Octynol                     | .51                                 | 12.73                 |
| Alkyl Pyridines HB                | .11                                 | 2.87                  |
| Formaldehyde (55%)<br>in Methanol | .60                                 | 15.00                 |
| Diacetone Alcohol                 | .42                                 | 10.46                 |

A further preferred composition of the present invention, sometimes referred to herein as composition E is as follows:

| Compound           | Composition E<br>Parts by<br>Volume | Per Cent<br>By Volume |
|--------------------|-------------------------------------|-----------------------|
| CRA                | 1.00                                | 25.0                  |
| Propargyl Alcohol  | 1.38                                | 34.4                  |
| Ethyl Octynol      | 0.14                                | 3.4                   |
| Alkyl Pyridines HB | 0.11                                | 2.8                   |
| Diacetone Alcohol  | 0.41                                | 10.3                  |
| Normal Propanol    | 0.96                                | 24.1                  |

A number of laboratory tests were conducted wherein the preferred blends of this invention, compositions A, B, C, D, and E, were tested at various temperatures, in various amounts with various aluminum alloys, under static conditions and dynamic conditions, in various hydrochloric acid solutions.

#### PROCEDURE FOR STATIC TESTS

In these tests, the acid solutions were mixed by diluting 20° Be' HCL with water to the desired concentrations. A portion of each acid solution was then titrated with a standard base solution to ascertain the exact acid concentration. The various acid solutions were prepared in advance in sufficient quantities to complete an entire series of tests with the same batch of acid. Corrosion coupons of various types of aluminum were ordered in sufficient quantities to complete a series of tests on the same batch of coupons. The coupons were cleaned as follows: Scrubbed by hand with a fine nylon brush in a detergent containing a pumice, rinsed, dipped in acetone to remove the access water and then

dipped in alcohol and allowed to dry. They were then weighed to the nearest milligram and stored in a desiccator until time for use.

Tests were conducted at various temperatures.

The acid solution was poured into glass bottles in sufficient quantity to approximate the specific acid volume to coupon surface area ratio that was desired. The quantity of acid used was dependent upon the surface area of the coupon to be tested. In most of the static tests, a 25 cc./in.<sup>2</sup> acid volume to coupon surface area ratio was used. After the desired amount of acid was poured into the bottles, the inhibitor composition was added with a hypodermic syringe, with the anionic surface active agent being added first separately and stirred with a glass rod, and then the other compounds in the particular inhibitor composition tested added and stirred with a glass rod. The inhibited acid solution was then placed in a water bath which had been set at a predetermined temperature and allowed to pre-heat for 20 minutes. After this time, the coupons were placed in the preheated inhibited acid solutions. The coupons were left in the acid solutions for the specified test time, then removed, neutralized, recleaned, rinsed, dipped in acetone and then alcohol, allowed to dry, and then reweighed.

#### PROCEDURE FOR DYNAMIC TESTS

The acid solutions in these tests were mixed and titrated in the same manner as outlined above for the static tests. In these tests 1 inch OD aluminum alloy tubing was cut into test specimens each measuring 6 inches. The specimens were cleaned by scrubbing by hand with a fine Nylon brush and a detergent containing pumice, rinsed, dipped in acetone to remove the excess water, and then placed in a desiccator and allowed to come to room temperature. The specimens were then weighed to the nearest milligram and stored in a desiccator until time for use.

The scaled specimens which had been pre-weighed to the nearest milligram were prepared by stopping up one end of the specimen and filling the specimen with a sealing solution. The sealing solution was calcium bicarbonate solution prepared by reacting a ten per cent calcium chloride solution with a sixteen per cent ammonium bicarbonate solution. The specimens containing the sealing solutions were then placed in an oven set at a temperature of 200°F. The sealing solution was allowed to evaporate leaving a calcium carbonate scale on the test specimens. The scaled specimens were then re-weighed to the nearest milligram and stored in a desiccator until time for use. All of these tests were conducted in a closed acid circulating system which had been calibrated to a desired velocity of acid flow.

The acid solution was poured into a glass bottle in sufficient quantity to approximate the specific acid volume-to-specimen surface area ratio that was desired. In most of these tests a 123 cc./in.<sup>2</sup> volume to specimen surface area ratio was used. After the desired amount of acid was poured into the bottles, the inhibitor was added with a hypodermic syringe, the anionic surface active agent being combined first and stirred with a glass rod, and then the other compounds in the composition tested were combined and stirred.

The flow rate of the system was calibrated by using a flow meter to measure flow and a variable resistor to regulate the speed of a circulating pump. The temperature of the acid solution was maintained at the desired

temperature for each test by use of a hot plate which was controlled with a Tele-Thermometer. The speci-

From the above Table it can be seen that best results were obtained with CRA in composition D.

TABLE II

COMPARISON OF VARIOUS ACETYLENIC ALCOHOLS  
AND  $C_{11}H_{22}SO_4Na$  (CRA) MIXTURES WITH COMPOSITION A

|                                  |                                                                       |                                                                 |                                                                             |                                                       |
|----------------------------------|-----------------------------------------------------------------------|-----------------------------------------------------------------|-----------------------------------------------------------------------------|-------------------------------------------------------|
| Type of Test                     | Dynamic                                                               |                                                                 |                                                                             |                                                       |
| Test Temp.                       | 150°F.                                                                |                                                                 |                                                                             |                                                       |
| Test Time                        | 6 hours                                                               |                                                                 |                                                                             |                                                       |
| Metal Type                       | Aluminum Alloy-3003 H14                                               |                                                                 |                                                                             |                                                       |
| Corrodent                        | 5% HCl                                                                |                                                                 |                                                                             |                                                       |
| Velocity                         | 1 ft./sec.                                                            |                                                                 |                                                                             |                                                       |
| Pressure                         | Atmospheric                                                           |                                                                 |                                                                             |                                                       |
| Surface Active Agent             | CRA                                                                   |                                                                 |                                                                             |                                                       |
| Acid Volume - Surface Area Ratio | 123cc/in. <sup>2</sup>                                                |                                                                 |                                                                             |                                                       |
| Acetylenic                       | Volume<br>Per Cent<br>Concentration<br>of CRA Surface<br>Active Agent | Volume<br>Per Cent<br>Concentration<br>of Acetylenic<br>Alcohol | Volume<br>Per Cent<br>Concentration<br>of Total<br>Inhibitor<br>Composition | Corrosion<br>Rate in<br>Lbs./Ft. <sup>2</sup><br>/Day |
| Propargyl<br>Alcohol             | 0.3                                                                   | 0.7                                                             | 1.0                                                                         | 0.0087                                                |
| Methyl<br>Butynol                | 0.3                                                                   | 0.7                                                             | 1.0                                                                         | 0.0860                                                |
| Hexynol                          | 0.3                                                                   | 0.7                                                             | 1.0                                                                         | 0.0066                                                |
| Composition A                    |                                                                       |                                                                 | 1.0                                                                         | 0.0016                                                |

mens were exposed to the circulating acid solution for the specified time, then removed, neutralized, cleaned, rinsed, dipped in acetone, allowed to dry, and then reweighed.

In both the static tests and dynamic tests the loss in weight of the coupons and/or specimens was multiplied times a calculated factor to convert the loss in weight to lbs./ft.<sup>2</sup>/24 hrs. The factor was calculated as follows:

$$\frac{144 \text{ in.}^2}{\text{ft.}^2} = \text{factor}$$

$$454 \frac{\text{g.}}{\text{lb.}} \times \text{Surface Area of Specimen-in.}^2$$

$$\times \text{Test Time-hrs.} \times \frac{1 \text{ day}}{24 \text{ hrs.}}$$

Example: Test time, 6 hours, surface area of coupon 4.0 in.<sup>2</sup> then

$$144/454 \times 4.0 \times (6/24) = 0.317 \text{ lb./ft.}^2/\text{day}$$

The results of these tests are set forth below:

TABLE I

COMPARISON OF VARIOUS ANIONIC

SURFACE ACTIVE AGENTS

|                                 |                         |
|---------------------------------|-------------------------|
| Type of Test                    | Static                  |
| Test Temperature                | 125°F.                  |
| Test Time                       | 4 hrs.                  |
| Metal Type                      | Aluminum Alloy-3003     |
| Corrodent                       | 5% HCl                  |
| Pressure                        | Atmospheric             |
| Acid Volume-Surface Area Ratio: | 25 cc./in. <sup>2</sup> |

| Inhibitor                                             | Volume Per Cent<br>Concentration<br>of Inhibitor | Corrosion<br>Rate in Lbs./Ft. <sup>2</sup><br>/day |
|-------------------------------------------------------|--------------------------------------------------|----------------------------------------------------|
| None                                                  | None                                             | 0.775                                              |
| CRA                                                   | 0.1                                              | 0.368                                              |
| Composition D                                         | .4                                               | 0.004                                              |
| Alkyl Taurate                                         | 0.1                                              | 0.097                                              |
| Alkyl Phosphate                                       | 0.1                                              | 0.124                                              |
| Alkyl Sulfate                                         | 0.1                                              | 0.136                                              |
| Composition D w/<br>Alkyl Taurate<br>in lieu of CRA   | 0.4                                              | 0.025                                              |
| Composition D w/<br>Alkyl Phosphate<br>in lieu of CRA | 0.4                                              | 0.072                                              |
| Composition D w/<br>Alkyl sulfate<br>in lieu of CRA   | in<br>0.4                                        | 0.008                                              |

As can be seen from the above data Composition A achieved the best result but relatively good results were also achieved with the other acetylenic alcohols tested.

TABLE III

INHIBITOR COMPOSITION B-CORROSION RATES  
FOR VARIOUS ACID STRENGTHS AND TEMPERATURE

|                                                   |                                   |                        |                                                     |
|---------------------------------------------------|-----------------------------------|------------------------|-----------------------------------------------------|
| Type of Test                                      | Dynamic                           |                        |                                                     |
| Test Time                                         | 6 Hours                           |                        |                                                     |
| Metal Type                                        | Aluminum<br>Alloy-3003 H14        |                        |                                                     |
| Velocity                                          | 1 ft./sec.                        |                        |                                                     |
| Pressure                                          | Atmosphere                        |                        |                                                     |
| Acid Volume-Surface Area Ratio:                   | 123cc./in. <sup>2</sup>           |                        |                                                     |
| Volume Per Cent<br>Concentration<br>Composition B | Corrodent<br>(Volume<br>Per Cent) | Test<br>Temp.<br>(°F.) | Corrosion<br>Rate in Lbs.<br>/ft. <sup>2</sup> /day |
| 1.0                                               | 5% HCl                            | 150                    | 0.0014                                              |
| 1.0                                               | 7½% HCl                           | 150                    | 0.0019                                              |
| 1.0                                               | 10% HCl                           | 150                    | 0.0076                                              |
| 1.0                                               | 5% HCl                            | 175                    | 0.0023                                              |
| 1.0                                               | 7½% HCl                           | 175                    | 0.0056                                              |
| 1.0                                               | 10% HCl                           | 175                    | 0.0072                                              |

Two specimens were subjected to the scaling process described above for the purpose of determining the amount of corrosion caused by scaling alone. After the scale was laid down on two specimens it was removed by brushing the specimens with a soft brush in warm water. The specimens were weighed before scaling and after the scale had been removed in order to determine weight loss due to the scale. Table IV shows the results of these tests.

Corrosion tests were conducted with inhibitor composition B in 5 per cent, 7½ per cent and 10 per cent hydrochloric acid solutions at 150°F. on specimens that contained a calcium carbonate scale layed down on the specimens as described above. These tests were conducted to determine if the inhibitor system would protect the aluminum surface once the scale had been removed by the acid. Table V reflects the results of these tests. The corrosion rates reported in this table have been corrected to reflect only the amount of corrosion that occurred from the acid solutions. The average

weight loss from the scaling process reflected in Table IV was deducted from the weight loss obtained with scaled specimens contacted by the acid solutions so that the reported corrosion rates in Table V reflect only the corrosion resulting from the inhibited acid solutions.

TABLE IV

| CORROSION OF SPECIMENS DUE TO SCALING |                       |                    |                        |                           |
|---------------------------------------|-----------------------|--------------------|------------------------|---------------------------|
| Specimen                              | Metal Type            |                    | Aluminum Alloy-3003H14 |                           |
|                                       | Original Wt. in Grams | Final Wt. in Grams | Wt. Loss In Grams      | Average Wt. Loss In Grams |
| No. 1                                 | 51.800                | 51.791             | 0.009                  |                           |
| No. 2                                 | 51.757                | 51.750             | 0.007                  | 0.008                     |

TABLE V

| INHIBITOR COMPOSITION B CORROSION OF SCALED SPECIMENS |                                                                |                                            |                                              |  |
|-------------------------------------------------------|----------------------------------------------------------------|--------------------------------------------|----------------------------------------------|--|
| Type of Test                                          | Dynamic 150°F., 6 hours                                        |                                            |                                              |  |
| Test Temp.                                            | Aluminum                                                       |                                            |                                              |  |
| Test Time                                             | Alloy-3003 H14 containing a CaCO <sub>3</sub> Scale 1 ft./sec. |                                            |                                              |  |
| Metal Type                                            | Atmospheric                                                    |                                            |                                              |  |
| Acid Velocity                                         | 123 cc./in. <sup>2</sup>                                       |                                            |                                              |  |
| Pressure                                              |                                                                |                                            |                                              |  |
| Acid Volume-Surface                                   |                                                                |                                            |                                              |  |
| Area Ratio:                                           |                                                                |                                            |                                              |  |
| Volume Per Cent Concentration of Composition B        | Corrodent (Volume Per Cent)                                    | Weight of CaCO <sub>3</sub> Scale in Grams | Corrosion Rate in Lbs./Ft. <sup>2</sup> /Day |  |
| 1.0                                                   | 5% HCl                                                         | 5.896                                      | 0.0037                                       |  |
| 1.0                                                   | 7½% HCl                                                        | 5.695                                      | 0.0064                                       |  |
| 1.0                                                   | 10% HCl                                                        | 5.821                                      | 0.0095                                       |  |

As can be seen by comparing Table III with Table IV very little additional corrosion took place as a result of the calcium carbonate scale, and the inhibitor system was very effective in protecting the aluminum specimen surface once the scale had been removed by the corrodent.

TABLE VI

| INHIBITOR COMPOSITION C- CORROSION RATES FOR VARIOUS ALUMINUM ALLOYS |                         |  |  |  |
|----------------------------------------------------------------------|-------------------------|--|--|--|
| Type of Test                                                         | Static 125°F.           |  |  |  |
| Test Temp.                                                           | 4 hours                 |  |  |  |
| Test Time                                                            | 5% HCl                  |  |  |  |
| Corrodent                                                            | Atmospheric             |  |  |  |
| Pressure                                                             | 25 cc./in. <sup>2</sup> |  |  |  |
| Acid Volume-Surface Area Ratio:                                      |                         |  |  |  |

| Aluminum      | Volume Per Cent Concentration of Composition C | Corrosion Rate in Lbs./Ft. <sup>2</sup> /Day |
|---------------|------------------------------------------------|----------------------------------------------|
| AA-179 (Cast) | None                                           | 0.820                                        |
| AA-179 (Cast) | 0.4                                            | 0.006                                        |
| AA-1100       | None                                           | 2.135                                        |
| AA-1100       | 0.4                                            | 0.003                                        |
| AA-2011       | None                                           | 1.212                                        |
| AA-2011       | 0.4                                            | 0.013                                        |

|         |      |       |
|---------|------|-------|
| AA-2017 | None | 2.840 |
| AA-2017 | 0.4  | 0.004 |
| AA-2024 | None | 1.145 |
| AA-2024 | 0.4  | 0.004 |
| AA-2117 | None | 3.121 |
| AA-2117 | 0.4  | 0.005 |
| AA-3003 | None | 0.775 |
| AA-3003 | 0.4  | 0.001 |
| AA-4043 | None | 2.870 |
| AA-4043 | 0.4  | 0.006 |
| AA-5005 | None | 0.298 |
| AA-5005 | 0.4  | 0.000 |
| AA-5052 | None | 0.608 |
| AA-5052 | 0.4  | 0.001 |

|         |      |       |
|---------|------|-------|
| AA-5056 | None | 1.300 |
| AA-5056 | 0.4  | 0.007 |
| AA-6053 | None | 0.094 |
| AA-6053 | 0.4  | 0.004 |
| AA-6061 | None | 1.323 |
| AA-6061 | 0.4  | 0.000 |
| AA-6063 | None | 0.626 |
| AA-6063 | 0.4  | 0.002 |

TABLE VII

| INHIBITOR COMPOSITION D-CORROSION RATES FOR VARIOUS ALUMINUM ALLOYS |                                                |                                              |
|---------------------------------------------------------------------|------------------------------------------------|----------------------------------------------|
| Type of Test                                                        | Static 125°F.                                  |                                              |
| Test Temp.                                                          | 4 hours                                        |                                              |
| Test Time                                                           | 5% HCl                                         |                                              |
| Corrodent                                                           | 3.065 ft/sec.                                  |                                              |
| Velocity                                                            | Atmospheric                                    |                                              |
| Pressure                                                            |                                                |                                              |
| Acid Volume-Surface Area Ratio:                                     | 181 cc./in. <sup>2</sup>                       |                                              |
| Type of Aluminum                                                    | Volume Per Cent Concentration of Composition D | Corrosion Rate in Lbs./Ft. <sup>2</sup> /Day |
| AA-3003                                                             | None                                           | Completely Dissolved                         |
| AA-3003                                                             | .55                                            | 0.015                                        |
| AA-5005                                                             | None                                           | 1.07                                         |
| AA-5005                                                             | .55                                            | 0.0008                                       |
| AA-6061                                                             | None                                           | Completely Dissolved                         |
| AA-6061                                                             | .55                                            | 0.013                                        |

TABLE VIII

| INHIBITOR COMPOSITION E-CORROSION RATES FOR VARIOUS ALUMINUM ALLOYS BY VARIOUS ACID SOLUTIONS AT VARIOUS TEMPERATURES |                         |                             |                                                |                                              |
|-----------------------------------------------------------------------------------------------------------------------|-------------------------|-----------------------------|------------------------------------------------|----------------------------------------------|
| Type of Test                                                                                                          | Static 4 hours          |                             |                                                |                                              |
| Test Time                                                                                                             | Atmospheric             |                             |                                                |                                              |
| Pressure                                                                                                              | 25 cc./in. <sup>2</sup> |                             |                                                |                                              |
| Acid Volume-Surface Area Ratio:                                                                                       |                         |                             |                                                |                                              |
| Type of Aluminum                                                                                                      | Test Temp.              | Corrodent (Volume Per Cent) | Volume Per Cent Concentration of Composition E | Corrosion Rate in Lbs./ft. <sup>2</sup> /Day |
| AA-3003                                                                                                               | 125°F.                  | 5% HCl                      | 0.4                                            | 0.001                                        |
| AA-5005                                                                                                               | 125°F.                  | 5% HCl                      | 0.4                                            | 0.001                                        |
| AA-3003                                                                                                               | 125°F.                  | 7.5% HCl                    | 0.4                                            | 0.002                                        |

TABLE VIII.—Continued

## INHIBITOR COMPOSITION E-CORROSION RATES FOR VARIOUS ALUMINUM ALLOYS BY VARIOUS ACID SOLUTIONS AT VARIOUS TEMPERATURES

| Type of Test     | Test Time | Pressure                          | Acid Volume-Surface Area Ratio                             | Static<br>4 hours                       | Atmospheric<br>25 cc./in. <sup>2</sup> |
|------------------|-----------|-----------------------------------|------------------------------------------------------------|-----------------------------------------|----------------------------------------|
| Type of Aluminum | Test Temp | Corrodent<br>(Volume<br>Per Cent) | Volume<br>Per Cent<br>Concentration<br>of<br>Composition E | Corrosion<br>Rate in Lbs.<br>/ft. 2/Day |                                        |
| AA-5005          | 125°F.    | 7.5% HCl                          | 0.4                                                        | 0.002                                   |                                        |
| AA-3003          | 125.20 F. | 10% HCl                           | 0.4                                                        | 0.002                                   |                                        |
| AA-5005          | 125°F.    | 10% HCl                           | 0.4                                                        | 0.002                                   |                                        |
| AA-3003          | 150°F.    | 5% HCl                            | 0.4                                                        | 0.001                                   |                                        |
| AA-5005          | 150°F.    | 5% HCl                            | 0.4                                                        | 0.001                                   |                                        |
| AA-3003          | 150°F     | 7.5% HCl                          | 0.4                                                        | 0.002                                   |                                        |
| AA-5005          | 150°F.    | 7.5% HCl                          | 0.4                                                        | 0.002                                   |                                        |
| AA-3003          | 150°F.    | 10% HCl                           | 0.4                                                        | 0.002                                   |                                        |
| AA-5005          | 150°F.    | 10% HCl                           | 0.4                                                        | 0.002                                   |                                        |

TABLE IX

## COMPARISON OF INHIBITOR COMPOSITIONS A AND B

|                                 |                         |
|---------------------------------|-------------------------|
| Type of Test                    | Dynamic                 |
| Test Temp.                      | 150°F.                  |
| Test Time                       | 6 hours                 |
| Corrodent                       | 5% HCl                  |
| Metal Type                      | AA-3003                 |
| Pressure                        | Atmospheric             |
| Acid Volume-Surface Area Ratio: | 123 cc/in. <sup>2</sup> |

  

| Inhibitor Composition | Volume Per Cent Concentration of Inhibitor Composition | Corrosion Rate in Lbs/Ft <sup>2</sup> /Day |
|-----------------------|--------------------------------------------------------|--------------------------------------------|
| A                     | 1.0                                                    | 0.0016                                     |
| B                     | 1.0                                                    | 0.0014                                     |

As can be seen from the above data the particular composition of the present invention which should be used for a particular application to obtain the best protection depends on the aluminum alloy to be protected, the strength of the acid solution to be employed, and temperatures to be encountered.

TABLE X

## CORROSION RATES OF VARIOUS ACID SOLUTIONS WITH AND WITHOUT COMPOSITION D

|                                                                   |                                        |                                                     |  |
|-------------------------------------------------------------------|----------------------------------------|-----------------------------------------------------|--|
| Type of Test                                                      | ASTM D-117                             |                                                     |  |
| Test Temp.                                                        | 125°F.                                 |                                                     |  |
| Test Time                                                         | 4 hours                                |                                                     |  |
| Metal Tested                                                      | AA-3003 Aluminum                       |                                                     |  |
| Pressure                                                          | Atmospheric                            |                                                     |  |
| Acid Volume-Surface Area Ratio:                                   | 25 cc/in. <sup>2</sup>                 |                                                     |  |
| <b>Volume Per Cent<br/>Concentration<br/>of<br/>Composition D</b> | <b>Corrodent<br/>(Volume Per Cent)</b> | <b>Corrosion Rate<br/>in Lbs/Ft<sup>2</sup>/Day</b> |  |
| 0                                                                 | 5% Sulfuric Acid                       | 0.005                                               |  |
| 0.4                                                               | 5% Sulfuric Acid                       | 0.004                                               |  |
| 0                                                                 | 5% Acetic Acid                         | 0.001                                               |  |
| 0.4                                                               | 5% Acetic Acid                         | 0.0008                                              |  |
| 0                                                                 | 5% Formic Acid                         | 0.0008                                              |  |
| 0.4                                                               | 5% Formic Acid                         | 0.0008                                              |  |
| 0                                                                 | 5% Hydrofluoric Acid                   | 1.11                                                |  |
| 0.4                                                               | 5% Hydrofluoric Acid                   | 1.06                                                |  |

As can be seen from the above table Inhibitor Composition D afforded some protection to the aluminum samples tested when combined with the various acid solutions tested, with the exception of Formic Acid which is not very corrosive to aluminum without inhibition.

From the above it may be seen that the inhibitor or inhibitor compositions of the present invention are operable when employed at temperatures as high as 175°F. in various acid concentrations. The corrosion which does occur is substantially uniform regardless of temperatures encountered and alloys protected. The corrosion inhibitor compositions provide long term protection at small concentrations and are particularly effective on aluminum and the various alloys thereof.

Applications in which the inhibitor of the present invention is particularly useful include cleaning of aluminum tanks, heat exchangers, pipe, etc., and preventing corrosion of aluminum tanks or vessels which must contain quantities of dilute acid.

The inhibitor of the present invention is preferably added to the acid in amounts by volume from about 0.05 per cent to 20 per cent. The amount of inhibitor required and the specific inhibitor composition will vary with the temperatures to be encountered, the particular aluminum alloy to be protected, and the strength or concentration of the acid solution used. The first part of the inhibitor, that is, the anionic surface active agent, should be combined first and mixed, and then the acetylenic compound, or mixture of acetylenic compound and non-acetylenic alcohol, or mixture of acetylenic compound, nitrogen compound, and non-acetylenic alcohol or mixture of acetylenic compound, nitrogen compound, and aldehyde, should be combined and mixed. The inhibitor composition may be added either to the water before acid is added or directly to the acid solution.

Broadly, the present invention relates to a new and improved corrosion inhibitor or composition for reducing the corrosive effect of aqueous acids on aluminum and the various alloys thereof consisting essentially of an anionic surface active agent and an acetylenic compound, or an anionic surface active agent and a synergistic blend of either an acetylenic compound and non-acetylenic alcohol or an acetylenic compound, a nitrogen or ammonia base compound and a non-acetylenic alcohol or aldehyde, in certain amounts of each.

**What is claimed is:**

1. A composition consisting essentially of:  
an aqueous hydrochloric acid solution having in the  
range of about 0.5 to 15% hydrochloric acid by  
weight of said solution;

a surface active agent selected from compounds represented by the general formula  $R_1SO_3X$  and mixtures thereof, wherein  $R_1$  is a saturated hydrocarbon radical having in the range of about eight to 25 carbon atoms and  $X$  is an alkali metal or ammonium; and

an acetylenic compound selected from compounds represented by the general formula



and mixtures thereof, wherein  $R_2$  and  $R_3$  are selected from alkyls and hydrogen and mixtures thereof, and further

wherein said hydrochloric acid solution is present in the range of about 98 to about 99.6% by weight of 5 said composition, said surface active agent is present in the range of about 0.06 to about 0.7% by weight of said composition, and said acetylenic compound is present in the range of about 0.26 to about 1.7% by weight of said composition. 10

2. The composition of claim 1 further consisting of an alcohol represented by the formula  $R_4OH$  wherein  $R_4$  is a radical selected from the group consisting of alkyls and ketones.

3. The composition of claim 2 further consisting of a 15 nitrogen base selected from the group consisting of mono-, di-, and trialkyl amines having from two to six carbon atoms in each alkyl moiety and 6-membered N-heterocyclic amines.

4. The composition of claim 1 wherein said surface active agent is represented by the chemical formula  $C_{13}H_{27}SO_3Na$ .

5. The composition of claim 4 wherein said acetylenic compound is selected from the group consisting of ethyl octynol, propargyl alcohol, methyl butynol, hexynol, and mixtures thereof.

6. The composition of claim 4 wherein said acetylenic compound is ethyl octynol.

7. The composition of claim 5 further consisting of 30 diacetone alcohol.

8. The composition of claim 7 further consisting of formaldehyde.

9. The composition of claim 7 further consisting of alkyl pyridines and normal propanol.

10. A method for protecting a metal selected from aluminum, aluminum alloys and mixtures thereof against corrosion by an aqueous hydrochloric acid solution in contact therewith, comprising contacting said metal with a composition consisting essentially of:

an aqueous hydrochloric acid solution having in the range of about 0.5 to 15% hydrochloric acid by weight of said solution;

a surface active agent selected from compounds represented by the general formula  $R_1SO_3X$  and mixtures thereof, wherein  $R_1$  is a saturated hydrocarbon radical having in the range of about eight to 25 carbon atoms and  $X$  is an alkali metal or ammonium; and

an acetylenic compound selected from compounds represented by the general formula



and mixtures thereof, wherein  $R_2$  and  $R_3$  are selected from alkyls and hydrogen and mixtures thereof; and further

wherein said hydrochloric acid solution is present in the range of about 98 to about 99.6% by weight of said composition, said surface active agent is present in the range of about 0.06 to about 0.7% by weight of said composition, and said acetylenic compound is present in the range of about 0.26 to about 1.7% by weight of said composition.

11. The method of claim 10 wherein said composition further consists of an alcohol represented by the formula  $R_4OH$  wherein  $R_4$  is a radical selected from the group consisting of alkyls and ketones.

12. The method of claim 11 wherein said composition further consists of a nitrogen base selected from the group consisting of mono-, di-, and trialkyl amines having from two to six carbon atoms in each alkyl moiety and 6-membered N-heterocyclic amines.

13. The method of claim 10 wherein said surface active agent is represented by the chemical formula  $C_{13}H_{27}SO_3Na$ .

14. The method of claim 13 wherein said acetylenic compound is selected from the group consisting of ethyl octynol, propargyl alcohol, methyl butynol, hexynol, and mixtures thereof.

15. The method of claim 13 wherein said acetylenic compound is ethyl octynol.

16. The method of claim 14 wherein said composition further consists of diacetone alcohol.

17. The method of claim 16 wherein said composition further consists of formaldehyde.

18. The method of claim 16 wherein said composition further consists of alkyl pyridines and normal propanol.

\* \* \* \* \*

UNITED STATES PATENT OFFICE  
CERTIFICATE OF CORRECTION

Patent No. 3,802,890 Dated April 9, 1974

Inventor(s) Billy R. Keeney

It is certified that error appears in the above-identified patent and that said Letters Patent are hereby corrected as shown below:

In Column 6, line 47, delete the word "sealing" and insert therefor --scaling--.

In Column 7, line 43, delete the line which reads  
"144/454 X 4.0 X (6/24) = 0.317 lb./ft.<sup>2</sup>/day" and insert  
-- $\frac{144}{454 \times 4.0 \times \frac{6}{24}} = 0.317 \text{ lb./ft.}^2/\text{day}$ --.

In Column 7, Table I, in the column entitled "Inhibitor" delete "Composition D w/ Alkyl sulfate lieu of CRA" and insert therefor --Composition D w/ Alkyl sulfate in lieu of CRA--. In the Column entitled "Volume Per Cent Concentration of Inhibitor" delete the word "in" which is reflected for Composition D w/Alkyl sulfate in lieu of CRA.

Signed and sealed this 17th day of September 1974.

(SEAL)

Attest:

McCOY M. GIBSON JR.  
Attesting Officer

C. MARSHALL DANN  
Commissioner of Patents